

## UNITED STATES PATENT OFFICE

ADOLF FRY, OF ESSEN, GERMANY, ASSIGNOR, BY MESNE ASSIGNMENTS, TO THE  
NITRALLOY CORPORATION, A CORPORATION OF DELAWARE

## STEEL ALLOY

No Drawing. Application filed May 6, 1927, Serial No. 189,457, and in Germany June 2, 1926. Renewed  
October 29, 1930.

The invention relates to steel alloys adapted for the manufacture of articles which are hardened in their marginal layers by nitrogenization.

- 5 For the manufacture of articles which are hardened by nitrogenization in their marginal layers according to the process disclosed in my Patent No. 1,487,554, I have previously disclosed the use of steel alloys which contain, either separately or in any desired combination, aluminium, chromium, manganese or silicon. The present invention has for its 10 object to afford the industry a group of quaternary and still more complex steel alloys which has not yet been disclosed, which alloys are easily produced, acquire great hardness in their marginal layers with relatively high hardness penetration when subjected to nitrogenization, and are distinguished further by particularly good properties of strength (in particular toughness and insensitiveness towards temper brittleness) and by their being well suited for heat treatment in large cross sections. This 15 object is attained according to the invention by using for the manufacture of the above-mentioned articles steel alloys which contain, either separately or in any desired combination, 1 to 8 per cent of silicon, manganese, 20 nickel, chromium, molybdenum, tungsten, vanadium, titanium or zirconium, less than 0.5 per cent of aluminium, and up to 0.7 per cent of carbon.

The following are representative examples 25 of alloy steels falling within the range above indicated and showing when nitrogenized the characterizing properties of surface hardness, hardness penetration, toughness and insensitiveness toward temper brittleness 30 above mentioned:

amounts to between 4 to 8 per cent, preferably such steel alloys may also be employed for the manufacture of the articles mentioned, which contain 0.5 to 2 per cent of aluminium. In this case it is proper to increase the percentage of aluminium, within the limits stated, in accordance with the total percentage of the other alloy constituents.

55 The subject matter of the next preceding paragraph forms the basis of my divisional application Serial No. 557,366 filed August 15, 1931.

60 What I claim and desire to secure by Letters Patent, is:—

1. An article hardened in its marginal layers by nitrogenization consisting of an alloy containing up to 0.7% of carbon, 1 to 8% of chromium, less than 0.5% of aluminium, and the principal portion of the remainder 65 iron.

70 2. An article hardened in its marginal layers by nitrogenization comprising an alloy containing up to 0.7% of carbon, 1 to 8% of at least one of the elements of the group, silicon, manganese, nickel, chromium, molybdenum, tungsten, vanadium, titanium and zirconium, less than 0.5% of aluminium, and the principal portion of the remainder being 75 iron.

80 The foregoing specification signed at Cologne, Germany, this 16th day of April, 1927.

ADOLF FRY.

85

| Example | C    | Al   | Cr   | Mn    | Mo    | Si   |
|---------|------|------|------|-------|-------|------|
| 1-----  | 0.29 | 0.19 | 1.64 | 0.42  | ----- | 0.32 |
| 2-----  | 0.31 | 0.45 | 1.68 | 0.45  | ----- | 0.34 |
| 3-----  | 0.3  | 0.25 | 2.0  | ----- | 0.30  | 0.4  |

90 If the total percentage of silicon, manganese, nickel, chromium, molybdenum, tungsten, vanadium, titanium or zirconium, either 95 separately or in any desired combination,

95

100